

May 20, 1941.

**McKINLEY STOCKTON**

2,242,796

## SYSTEM FOR COMMINUTING SOLIDS

Filed June 19, 1937



**MCKINLEY STOCKTON**  
*INVENTOR*

Paul W. Kuehne  
ATTORNEY

## UNITED STATES PATENT OFFICE

2,242,796

## SYSTEM FOR COMMINUTING SOLIDS

McKinley Stockton, Redmond, Oreg., assignor to  
 The Dicalite Company, Los Angeles, Calif., a  
 corporation of Delaware

Application June 19, 1937, Serial No. 149,187

3 Claims. (Cl. 83—94)

The object of my invention is to provide new and improved means for comminuting solids, particularly solids such as diatomaceous earth which have a fragile internal structure.

The invention comprises broadly a system in which the earth, originally in the large lumps in which it is taken from the deposit, is cracked by wedging forces, pressure or other suitable means into lumps of moderate size; in which a stream of the lumps is commingled with a stream of hot gases by which the earth is heated and deprived of water; in which the cooled gases and the water vapor evolved from the earth are separated from the dried lumps and discharged from the system, and in which the lumps of earth are finally, and only after substantially complete drying, introduced into a hammer mill, fan mill or other apparatus by which they are disintegrated and reduced to a powder by repeated impacts at high velocity.

In its preferred form the invention comprises the additional steps of an intermediate separation of spent gases and water vapor from the stream of lump earth prior to the completion of the drying thereof; the formation of the partially dried lump earth into a second stream, and the commingling of the earth stream with a second stream of hot gases to effect the drying of the lumps prior to their disintegration by impact.

It is well known to dry diatomaceous earth by bringing it into contact with a stream of hot gases, but heretofore this method of drying has been applied during the process of disintegration. For example, in Stockton Patent 1,611,791 a stream of hot gas is introduced into the suction of a hammer mill in which the lump earth from a set of cracking rolls is being disintegrated and a second hot gas stream into the suction of a fan mill in which the second disintegration is accomplished. Also in Cummins Patent 1,813,916 a stream of hot gas is introduced into the suction of a fan mill which produces the first disintegration and a second stream into the suction of a second fan mill in which the disintegration is completed. In both of these cases, and regardless of the relative position of the first impact mill, it is obvious that at least the first impact disintegration is performed on an earth which is incompletely, if at all, dried, and in fact these systems subject the earth to the forceful impacts required for partial disintegration before any material quantity of water is removed from the lumps of earth fed to them.

The advantages attending the drying of diatomaceous earth in lump form and prior to the

application of the pulverization step thereto may briefly be stated as follows:

Diatomaceous earth consists of an aggregation of the siliceous skeletons or casts of marine or lacustrine diatoms. In crude earths of good quality these casts, which are of microscopic size but of an elaborate structure, are in large part unbroken, and the quality of the products made from the crude depend to a great extent on the maintenance of this unbroken structure through the various manufacturing operations and particularly through the steps of drying and pulverization. The unbroken diatom structures behave like wool fibres, "felting" into a mass which is of extreme porosity and lightness and better adapted than perhaps any other known material to the filtration and clarification of liquids, while the breaking down of the diatom structures progressively reduces the porosity and increases the density of the mass until, when the degradation of the structures has been carried to the limit, the mass of crushed particles has substantially the properties of an amorphous siliceous mass and has entirely lost its usefulness as a filtering agent and for most other purposes.

Diatomaceous earth as it occurs in nature is usually water saturated and the crude earth as taken from the deposit often contains 50% or more by weight of free water. This water is strongly retained and air drying under favorable summer conditions will seldom reduce the moisture content below about 8% after 30 days' exposure, while in winter drying practically ceases. The cost of handling and the uncertainty of result make the air drying step economically unattractive and it is customary to dry the crude earth by the application of superatmospheric temperatures.

The wet earth as taken from the deposit is relatively very heavy and the presence of water and often of traces of clay render it tough and even slightly plastic. Per contra, lumps of dried diatomaceous earth are extremely light and very brittle. It follows that while the wet earth may be cracked down to lumps of moderate size (as for example such as will pass through a 2" mesh screen) with relatively small damage to the diatom structure, the attempt to reduce it to powder from the wet condition either by crushing, grinding or impact pulverization results in a very serious depreciation of the structure and of the value of the product, while in the dried form it may be disintegrated to powder in hammer mills or fan mills with much less depreciation. In the practice of the process herein disclosed I have,

in fact, greatly improved both the quality and the yield of the types of product used for filtration of liquids and have decreased the proportionate yield of relatively valueless "fines" or broken diatoms.

Lump diatomaceous earth has heretofore been dried prior to comminution, but only by methods each of which has serious disadvantages. Air drying is costly, uncertain, and restricted to favorable seasons and climatic conditions. Drying by indirect heat, as in steam jacketed or fire heated pans, is prohibitively wasteful of fuel. Drying by direct contact with counterflowing fire gases, as in a rotary kiln or on a rabbled hearth, involves the use of costly apparatus, a heavy power consumption, and a waste of fuel due to the low firing temperature required to avoid overheating of the dried lumps which encounter the hottest gases.

I have discovered that, when certain precautions are taken in the arrangement and operation of the apparatus, it is possible to apply the principle of concurrent, direct contact heating to the drying of relatively large lumps of diatomaceous earth and other materials of which it is desired to preserve the internal structure through a comminuting step, and that by proceeding in the manner below described I obtain a product of improved quality, in apparatus of materially reduced cost, and with a minimum consumption of fuel. These precautions will be described in connection with the following descriptions of exemplary apparatus suited to the practice of the methods of the invention, these descriptions referring to the attached drawing which illustrates in a diagrammatic manner an assemblage of apparatus particularly adapted to the treatment of massive, compacted earths substantially free from organic matter.

Referring first to Fig. 1, 1—1 is a pair of toothed rolls revolving toward each other and supplied with large lumps of the earth as taken from the deposit or as partially air dried if so preferred. These rolls, or a jaw or other crusher which might be substituted for them, crack the earth into lumps of moderate size. These are conventional methods for accomplishing the first size reduction. It is desirable to exercise the least possible crushing effect on the wet earth, and for this reason I prefer toothed rolls, which exercise a wedging force, rather than jaw crushers. No rule can be laid down for the size of the lumps as the preferred size will depend on the proportion of original water and also the relative freedom of drying, this being in turn governed by the presence or absence of clay and other factors. In a general way it may be said that the crude lumps should range downwardly from a maximum of 2", though this is by no means a limiting condition and the most favorable size range for any given deposit will be found only by experiment.

The cracked earth may conveniently be caused to fall on a tilting apron 2 by which it is diverted into one or the other of the lump storage bins 3—3, from one or the other of which a continuous stream of the lumps is delivered on to a belt conveyor 4 by means of any feeding device indicated at 5—5. The conveyor delivers this stream of earth into a hopper 6 which is provided with a seal valve, indicated at 7, for delivering the earth into the drying system while preventing inflow or outflow of air or gas.

A combustion chamber or furnace 8 is provided with a gas, oil, or other burner 9 and an air inlet 75

10 pipe 10 having a valve or damper 11 to control the flow of primary air to the burning fuel. This furnace may be operated either above or below atmospheric pressure, as may be preferred, though in the drawing it is illustrated as operating under suction.

The gases produced by perfect combustion in the furnace may be too hot to apply to the lumps of earth and in such cases should be tempered by admixture with a cold or a cooler gas. Air for this purpose may be drawn into the combustion space of the furnace through pipe 10 or preferably may be introduced into the gas stream flowing through the furnace outlet by means of branch pipe 12 controlled by valve 13.

The hot gaseous mixture, brought to the optimum temperature hereinafter defined, enters the drying tube 14 where it encounters the stream of earth passing through seal valve 7. The combined stream traverses the length of tube 14, in which interchange of heat between the gases and the earth is effected, and enters a cyclone or other separator 15 in which the earth is collected. The spent gas and water vapor are removed from the separator through pipe 16 by means of a suction blower 17 and are discharged into the atmosphere or elsewhere as may be desired.

The blower 17 provides the reduction in pressure by which the stream of gases and earth is drawn through the drying tube. It is fully equivalent to operate the drying system at a slight superatmospheric pressure instead of at subatmospheric as shown.

The earth collecting in separator 15 is continuously discharged through a seal valve 18 into a drying tube 19 which is supplied with hot gases from combustion of fuel in furnace 20, which may be equipped as described in connection with furnace 8. Air for tempering the combustion gases may if required be drawn into the furnace outlet through a pipe 21 controlled by valve 22. Under some conditions the supply of fuel to furnace 20 may be discontinued or this unit may be omitted from the system, air alone being admitted to tube 19 as will be described.

The stream of gases and earth traverses the length of drying tube 19, in which the interchange of heat between the gases and the earth is effected, and enters the suction of a fan mill 22 in 50 which the earth, which at this stage is substantially completely dried, is pulverized to the desired fineness, ordinarily that required in a filter-aid. The pulverized earth, spent gases, and water vapor pass through pipe 23 into a cyclone or other separator 24 from which the gases and vapors are vented through pipe 25 to the atmosphere or elsewhere. The pulverized earth, the final product of the operation, collects in the separator and may be withdrawn as required by means of the screw conveyor 26.

It is the spirit of this invention to substantially completely dry the earth before it is submitted to the step of pulverization or disintegration by impact, as in a fan mill or hammer mill. Substantially complete drying should be interpreted as drying to the moisture content permissible in the pulverized final product, or that which renders the earth so friable that it may be disintegrated without material damage to the diatom structure. Ordinarily this will be from 3% to 8% by weight of uncombined water, though in cases of exceptionally pure and friable earths it may be even as high as 15%.

The above degree of dessication may, under favorable conditions, be produced by the use of

hot gases in only the first pass, i. e., in drying tube 14. In this case, as above said, secondary furnace 20 is not operated and air is admitted at valve 22 only to carry the dried earth from separator 15 into fan mill 22.

The drying tubes, and particularly the primary tube 14, should be extended to the greatest possible length if it is desired to secure the maximum of fuel economy. In these tubes the flow of gases and earth is concurrent and the temperature head from gas to earth diminishes progressively toward the tube outlet, making heat transfer relatively slow at this end of the tube. The lengths of the tubes are minimized in the drawing. In practice they are proportioned to the quantity of water to be evaporated, the volume of gas per pound of earth fed, the permissible initial temperature of the gas and the velocity of the gas stream.

Because the earth first encounters the hot gases while in the wet condition and in the form of lumps substantially free from fine particles, it is possible to utilize gases at a much higher initial temperature than is possible either in countercurrent heating (as in a rotary kiln or on a hearth) or where the gas is introduced into the disintegrating device (as in Stockton 1,611,791 or in Cummins). The rapid evaporation of water from the surface of the lump and the simultaneous diffusion of water from the interior or the exterior portions effectively protect the superficial portions of the lump from overheating until a considerable part of the water has been evaporated, at which time the gases have cooled below the danger point. It is therefore possible to supply primary drying tube 14 with extremely hot gases, as of the order of 1800° to 2000° F., such as have heretofore been used only for the calcination of previously pulverized earth. These initial temperatures may be used without the slightest danger of glazing or sintering the surfaces of the lumps.

With sufficient extension of the primary drying tube it is possible to reduce the discharged gas-vapor mixture to 200° or even to 150° F. Evaporation of water from the earth continues down to these low temperatures because of the high ratio of fixed gas to water vapor even at the outlet end of the tube. Because of this wide range between initial and final temperatures and because of the small spread between final temperature and atmosphere, this stage of the process is extremely economical of fuel, requiring but little more heat supply than that rendered latent in evaporating the water.

In some cases, as for instance where the water percentage is excessive or the water is strongly retained because of clay or gelatinous silica in the earth, it may be impossible to dry to the required final percentage in the primary tube alone without unduly reducing its throughput. In such cases I utilize the secondary drying stage above described, supplying hot gases to secondary drying tube 19. As the earth entering this stage is much reduced in water content, it is advisable to maintain the hot gas supply at a materially lower initial temperature, as for example from 800° to 1000° F. The second drying stage discharges its vent gas at a higher temperature than the first stage and is necessarily less economical of fuel, but by reason of replacing the gas-vapor mixture existing at the tail end of the first stage with a dry gas at a higher temperature, a relatively small hot gas supply will complete the dessication of a large quantity of partially dried earth. The most

economical overall adjustment of the system is usually that in which the greatest possible proportion of the total water is removed in the first stage, even though this entails a moderate increase in temperature at the outlet of the primary tube.

It will be understood that the temperatures above recited are suggestive only and not limiting, and that they will be modified in the light of experience with different earths and under varying conditions.

The dried material finally entering fan mill 22 for disintegration still consists mainly of lumps, though these will usually be of smaller average size than those originally supplied to the primary drying tube. This reduction in average size is due mainly to cracking and spalling of the larger original pieces during drying, though some dust is formed and is vented from the separators with the spent gases. This dust may be collected in a bag-house or spray tower if it should constitute a nuisance. The amount of actual pulverization is small, as the impacts to which the lumps are subjected during their travel through the drying system are inappreciable as compared with the powerful blows to which they are subjected in fan or hammer mills.

At the point where the lumps enter the fan mill they are reduced to more or less one-half their original weight and density and, instead of being tough or incipiently plastic are extremely brittle. The force of the disintegrating impacts, in any given apparatus, is reduced in proportion to the reduction in weight and consequent inertia, but the fragility imparted to the lump by the removal of water (fragility of the lump as a whole, not of its constituent diatom structures) more than offsets this reduction in disintegrating force. The methods and apparatus above described thus render possible the retention of an increased proportion of the diatom structures in the unbroken condition, and correspondingly increase the value of the comminuted product while decreasing the cost of apparatus and the consumption of power and fuel.

The very striking advantages attending the use of the above described methods and apparatus are shown by the following figures for wet density of the comminuted product, for flow rate in filtering raw sugar solutions and for clarity of the filtrate. The first column shows the test figures for an earth milled in the manner shown in Fig. 1 of my U. S. Patent 1,611,791, in which the hot gases for drying are introduced directly into the suction of the mill in which the first comminution is effected. The second column shows the results with identical crude earth (and equal doses in the filtration tests) when dried and comminuted in the manner above described.

|                  | Old method | New method |
|------------------|------------|------------|
| Wet density----- | 19.5       | 15.2       |
| Flow rate-----   | 228        | 458        |
| Clarity -----    | G          | H          |

As will be seen, the density of the comminuted earth is reduced 22%, while for equal clarities the flow rate is almost exactly doubled. These are major advantages.

I claim as my invention:

1. The method of drying and comminuting crude diatomaceous earth which comprises: feeding lumps of said earth into a rapidly moving stream of hot fixed gases; maintaining said lumps and said gases in direct contact and in motion in a common substantially horizontal di-

rection until a desired proportion of the water content has been vaporized from said lumps; separating the partially dried lumps from said gas stream and rejecting said gas stream; feeding said separated lumps into a second rapidly moving stream of hot fixed gases; maintaining said lumps in direct contact with said second stream and in motion in a common substantially horizontal direction until said lumps are substantially completely dried, and pulverizing said lumps only after last said drying step.

2. The method of drying and comminuting crude diatomaceous earth which comprises: feeding lumps of said earth into a rapidly moving stream of hot fixed gases; maintaining said lumps and said gases in direct contact and in motion in a common substantially horizontal direction until said lumps of earth are substantially completely dried; separating said lumps from spent gases

5 and vapors and diverting said gases and vapors out of the system; suspending said lumps in a second gaseous stream, and pulverizing said lumps by repeated impacts while in suspension in said second stream and only after the completion of said substantial drying.

3. The method of drying and comminuting crude diatomaceous earth which comprises: feeding lumps of said earth into a rapidly moving stream of hot fixed gases; maintaining said lumps and said gases in direct contact and in motion in a common substantially horizontal direction until said lumps are substantially completely dried; separating said lumps from spent gases and vapors; suspending said lumps in a stream of air, and pulverizing said lumps by repeated impacts while in suspension in said air stream and only after the completion of said substantial drying.

MCKINLEY STOCKTON.